

May 4, 1971

F. E. GOULD ET AL

3,577,516

PREPARATION OF SPRAY ON BANDAGE

Filed Dec. 3, 1969

*Fig. 1.*



*Fig. 2.*



*Fig. 3.*



*Fig. 4.*



## 1

3,577,516

**PREPARATION OF SPRAY ON BANDAGE**  
Francis E. Gould, Princeton, and Thomas H. Shepherd,  
Hopewell, N.J., assignors to National Patent Develop-  
ment Corporation, New York, N.Y.  
Continuation-in-part of applications Ser. No. 567,856,  
July 26, 1966, now Patent No. 3,520,949, Ser. No.  
650,259, June 30, 1967, and Ser. No. 654,044, July 5,  
1967. This application Dec. 2, 1969, Ser. No. 881,376  
Int. Cl. A61L 15/00

U.S. Cl. 424—46

17 Claims

### ABSTRACT OF THE DISCLOSURE

A bandage is formed in situ on a wound by spraying on separately or simultaneously a hydrophilic water insoluble polymer and a high boiling plasticizer or solvent therefor. Preferably the polymer is a hydroxy lower alkyl acrylate or methacrylate. Medically active ingredients can be included in the composition.

The present application is a continuation-in-part of application Ser. No. 567,856 filed July 26, 1966 now Pat. 3,520,949 issued July 21, 1970; application Ser. No. 650,259, filed June 30, 1967 and now abandoned; and application Ser. No. 654,044, filed July 5, 1967.

The present application relates to spray-on bandages.

A spray-on bandage offers a convenient, easy method of protecting minor wounds, cuts and/or abrasions during the healing process, and avoids certain undesirable characteristics associated with the use of substrates coated with pressure sensitive adhesives and gauze pads; such as pain and peeling of hair during removal, disagreeable appearance, adhesion of the healing area to the gauze pad, etc.

The requirements for a fully acceptable spray-on bandage include the following:

- (1) It protects the wound from air borne bacteria and dirt.
- (2) It has moisture vapor permeability sufficient to prevent accumulation of aqueous fluid under the bandage.
- (3) It must be non-toxic and non-irritating to the skin.
- (4) It should not adhere to the wound area or permit infiltration by regenerating tissue.
- (5) It should not cause a burning or stinging sensation when applied.
- (6) It should not be water soluble or rendered tacky by contact with water to avoid dirt accumulation.
- (7) It should be readily removable when desired.

Prior art spray-on products suffer from a number of disadvantages with respect to the above criteria. Thus prior art materials having the desired moisture vapor permeability coupled with water resistance must be applied as a spray from alcohol or similar solvent solution which causes a strong burning sensation in the wound area.

It is an object of the present invention to develop a spray-on bandage having all seven of the above set forth desirable characteristics while avoiding the disadvantages of prior art spray-on bandages.

Still further objects and the entire scope of applicability of the present invention will become apparent from the detailed description given hereinafter; it should be understood, however, that the detailed description and specific

## 2

example, while indicating preferred embodiments of the invention, are given by way of illustration only, since various changes and modifications within the spirit and scope of the invention will become apparent to those skilled in the art from this detailed description.

It has now been found that these objects can be attained and a film forming action can be caused by applying a mixture of a powder of certain water insoluble, hydrophilic polymers having a high moisture vapor permeability with high boiling non-toxic polar "plasticizer" solvents therefore to, in effect, create a room temperature gelling "plastisol" which has high moisture vapor permeability, is sufficiently adherent to the skin to remain in place for extended periods of time, and adequately protects wound areas from contamination. Films produced by this technique are readily removed by soaking the bandages area in water for a few minutes which loosens the bond between the plastisol film and the skin. The film can then be readily pulled from the skin surface without discomfort.

The invention can be used to form spray-on bandages not only for human wounds but also is useful in the field of veterinary medicine for wounds on the skins of animals such as dogs, cats, sheep, cattle (e.g. to protect cows having mastitis on their teats), goats, pigs and horses and zoological animals such as lions, tigers, deer, zebra, etc.

Furthermore there can be incorporated in the films of the invention medically active ingredients which will diffuse from the film to the wound area over extended periods of time and keep the wound area free from infection, or provide local anesthesia or analgesia properties.

The medically active ingredients can be incorporated in the film by either (1) having them impregnated in the polymer or (2) mixing the active ingredient with the polymer powder, or (3) dissolving or dispersing the active ingredient in the high boiling plasticizer-solvent.

Polymer powders useful in this invention include polymers of hydroxy lower alkyl acrylates and methacrylates alone or copolymers with each other, e.g. copolymers of 1 to 99% of each. Such polymers include hydroxyethyl acrylate, hydroxyethyl methacrylate, hydroxy propyl acrylate and hydroxypropyl methacrylates. The preferred polymers are hydroxy lower alkyl methacrylates, especially hydroxyethyl methacrylate polymers.

There are also be used copolymers of the hydroxyalkyl acrylates and methacrylates with up to 50 weight percent of lower alkyl acrylates and methacrylates, e.g. methyl acrylate, ethyl acrylate, propyl acrylate, isopropyl acrylate, butyl acrylate, methyl methacrylate, ethyl methacrylate, isopropyl methacrylate and butyl methacrylate, hydroxy lower alkoxy lower alkyl acrylates and methacrylates, e.g. diethylene glycol monoacrylate, diethylene glycol mono methacrylate, dipropylene glycol mono acrylate, dipropylene glycol mono methacrylate, acrylamide, methacrylamide, N-methyl acrylamide, N-methyl methacrylamide, N-ethyl acrylamide, N-ethyl methacrylamide, N-propyl acrylamide, N-propyl methacrylamide, N-isopropyl acrylamide, N-isopropyl methacrylamide, lower alkoxy lower alkyl acrylates and methacrylates such as methoxyethyl acrylate, methoxyethyl methacrylate, ethoxyethyl acrylate and ethoxyethyl methacrylate, amine compounds, e.g. p-aminostyrene, 2-amino-4-vinyltoluene, diethylaminoethyl acrylate, diethylaminoethyl methacrylate, dimethylaminoethyl acrylate, dimethylaminoethyl methacrylate, t-butylaminoethyl methacrylate, piperidinoethyl

acrylate, 2-vinyl pyridine, dimethylaminopropyl methacrylate, diacetone acrylamide, diacetone methacrylamide, N-vinyl pyrrolidone.

The copolymerizable material should not be used in such amount as to reduce the compatibility of the hydroxalkyl acrylate or methacrylate with the solvent or plasticizer or render it either too soluble in water or reduce its hydrophilic properties too greatly.

Usually the hydroxalkyl acrylate or methacrylate is at least 80% by weight of the total monomers.

Useful, but less preferable, copolymers are prepared from lower alkyl acrylates and methacrylates, e.g. having 1 to 3 carbon atoms in the alkyl group such as methyl acrylate, ethyl acrylate, isopropyl acrylate, methyl methacrylate, ethyl methacrylate and propyl methacrylate with 30-80% of ethoxyethyl acrylate, methoxyethyl acrylate, methoxyethyl methacrylate, ethoxyethyl methacrylate, acrylamide, methacrylamide, n-alkyl substituted acrylamides and methacrylamides such as N-methyl acrylamide, N-propyl acrylamide, N-methyl methacrylamide and N-isopropyl methacrylamide and N-vinyl pyrrolidone. Also polymers of the alkyl acrylates and methacrylates with 30-50% of hydroxyethyl and hydroxy propyl acrylates and methacrylates are included in this less preferred category.

In addition to the monomer and monomer mixtures set forth above to prepare polymers there can be added to the monomer or monomer mixture up to 15% by weight of the total monomers of acrylic acid, methacrylic acid, itaconic acid, maleic acid or fumaric acid.

While in Shepherd patent 3,428,043 there is described the use of a bandage comprising a fabric having an infrequently cross-linked hydrophilic polymer combined therewith the polymers of the present invention unlike those set forth in the Shepherd patent are substantially devoid of cross-linking. Thus while the slight amount of cross-linking ethylene glycol dimethacrylate impurity (about 0.1 to 0.2%) normally present in hydroxyethyl methacrylate can be tolerated any cross-linking agent present should not be sufficient to interfere with compatibility of the hydrophilic polymer with the plasticizer-solvent so as to prevent plastisol formation or otherwise interfere with the formation of the bandage on the wound.

The presently most preferred polymer is Hydron S, a commercially available polymer of hydroxyethyl methacrylate. It is essentially a homopolymer except for the presence of a trace (about 0.1% by weight) of ethylene glycol dimethacrylates.

The main requirements of the polymers useful in the present invention are:

(1) Non-tackiness.  
(2) Sufficient hydrophilic character to possess moisture vapor permeability of at least 200 grams/sq. meter/24 hours/mil, preferably at least 500 grams/sq. meter/24 hours/mil.  
(3) Susceptibility to solvation (plastisol formation) by the useful polar plasticizer-solvents.

(4) Insolubility in water.  
(5) Sufficient friability to be able to be prepared as a finely divided powder, e.g. less than 100 mesh and preferably less than 200 mesh (Tyler Screen series).

Plasticizer-solvents useful for film formation in combination with the polymer-powders include water soluble polar compounds including glycols such as propylene glycol, ethylene glycol, trimethylene glycol, butanediol-1,3, butanediol-1,4, hexanediol-2,5, 2-methyl-2,4-pentanediol, heptanediol-2,4, 2-ethyl-1,3-hexanediol, diethylene glycol, triethylene glycol, tetraethylene glycols and other polyethylene glycols having a molecular weight up to 800 (e.g. hydroxy terminated polymers of ethylene oxide having average molecular weights of 200-800), dipropylene glycol, tripropylene glycol and other polypropylene glycols having molecular weights up to 900, propylene glycol monoethyl ether, mono acetin, tri(hydroxyethyl) citrate,

di(hydroxypropyl) oxalate, hydroxypropyl acetate, glyceryl triacetate, glyceryl tributylate, liquid sorbitolethylene oxide adducts, liquid glycerine-ethylene oxide adducts, diethylene glycol monomethyl ether, diethylene glycol monoethyl ether, ethylene glycol diacetate.

The ratio of the plasticizer-solvent to the polymer is not particularly critical and satisfactory results are obtained in the range of from 80%-20% polymer to 20%-80% plasticizer-solvent, more preferably 30-70% polymer to 70-30% plasticizer-solvent.

Unless otherwise indicated, all parts and percentages are by weight.

In practice, it has been found that a light application of the plasticizer-solvent to the skin followed by application of the polymer powder results in adherence of a sufficient quantity of the powder to the area wet with the plasticizer-solvent to result in a strong, tough, adherent film. The film can be built up to any desired thickness but is usually about 10 mils.

The spray-on bandage of this invention is most conveniently applied using aerosol spray techniques although a layer of liquid followed by a layer of polymer can be applied by brushing, dabbing, etc. The bandage may be applied by a 2-separate spray technique wherein the plasticizer-solvent is first applied, followed by application of the powder from a separate container. Alternatively, the powder and liquid may be applied simultaneously from separate aerosol cans and valves which have a common activating mechanism. In some cases the powder and liquid may be applied from the same can in which case, the presence of the propellant in the can prevents solvation and agglomeration of the powder by the plasticizer solvent.

Suitable propellants include those well known in the art. There can be used compressed gases such as carbon dioxide, nitrous oxide, nitrogen, liquified volatile hydrocarbons such as propane, n-butane, isobutane and 2-methyl butane, methylene chloride, vinyl chloride, fluorinated compounds including perhalogenated compounds and fluorinated hydrocarbons such as dichlorodifluoromethane (Freon 12), trichlorofluoromethane, 1,2-dichlorotetrafluoroethane, octofluorocyclobutane, chlorodifluoromethane, 1,1-difluoroethane, vinyl fluoride, vinylidene fluoride, 1-chloro-1,1-difluoroethane. The propellant should contain a substantial amount of volatile material boiling at not over 20° C., but there can also be present a significant amount of less volatile material boiling up to 50° C.

The invention will be understood best in connection with the drawings wherein:

FIG. 1 is a perspective view illustrating the spraying of the plasticizer-solvent according to the invention;

FIG. 2 is a perspective view showing the spraying of the polymer;

FIG. 3 is a view of the finishing bandage; and

FIG. 4 is a view of an alternative method according to the invention.

Referring more specifically to FIGS. 1 and 2 of the drawings there is shown a skin area 2, e.g. on the arm, having a cut 4 thereon. From aerosol can 6, there is directed a spray 8 of appropriate plasticizer-solvent, e.g. propylene glycol by means of propellant, e.g. dichlorodifluoromethane. After the spraying of the plasticizer-solvent is completed, there is then sprayed from aerosol can 10 powdered Hydron S 12 on top of the plasticizer-solvent. The Hydron S merges with the plasticizer-solvent to form the completed bandage 14 as a plastisol as shown in FIG. 3.

In the form of the invention illustrated in FIG. 4 a single aerosol can 16 is provided with a chamber 18 for the Hydron S and a separate chamber 20 for the propylene glycol plasticizer-solvent. When valve 22 is operated in the direction of the arrow, it releases the polymer 18 and plasticizer-solvent together with the propellant as shown to coat the wound 24 on skin 26 to provide a bandage.



## Example 11

The procedure of Example 10 was repeated replacing the hexachlorophene by 0.3 gram of Bacitracin (or anti-septic). The film formed on spraying showed good suppression upon a colony growth of streptococci. A spray on bandage was also produced on skin on the cheek.

## Example 12

The procedure of Example 10 was repeated replacing the hexachlorophene by 0.3 gram of cortisone. When the spray on bandage was formed on the skin good anti-inflammatory effect upon the skin was noted.

## Example 13

The procedure of Example 10 was repeated using 0.3 gram of Benzocaine (ethyl aminobenzoate, a local anesthetic) in place of the hexachlorophene. The resulting film showed good pain suppressing qualities upon abraded skin.

## Example 14

Any medically active ingredient that is soluble in ethanol or an ethanol-water mixture can be put into solution with Hydron S or other hydroxyethyl or hydroxypropyl methacrylate polymers. Such solutions are then dried to a solid by any method known to the art, e.g. tray drying, roller drying, vacuum drying, spray drying, and then reduced to sprayable powder form to produce an entrapped medically active ingredient.

For example, 9.0 grams of Hydron S plus 1 gram of Benzocaine were dissolved in 30 cc. of 95% ethanol. The solution was vacuum dried and the resulting polymer mix was pulverized to -270 to -325 mesh. This polymer mix was charged into an aerosol can as described in Examples 10 and 13. Upon spraying to form a bandage, the final film produced on the skin showed the same pain suppressing qualities as in Example 13 above.

## Example 15

If the medically active ingredient is soluble in the liquid phase of the system, it can be dissolved in that phase with results similar to those described in Examples 9-14.

For example a six ounce aerosol can was charged with 9.7 grams of Hydron S, -220 to -325 mesh and sealed with a codispensing valve and bag assembly. The bag chamber was then charged with a solution of 8 grams of propylene glycol containing 0.3 gram of hexachlorophene and 32 grams of Freon 12. The sprayed film produced the same suppression of a *Salmonella typosa* colony as in Example 10. A satisfactory spray-on bandage was also produced on skin having a wound therein.

Obviously the medicinally active ingredient can be added to both the polymer and the plastisol forming solvent or plasticizer.

What is claimed is:

1. In a method of forming a powdery bandage in situ on skin having a wound therein which is readily removable therefrom after soaking, the improvement comprising the steps of (a) applying, as a powder, a hydrophilic water insoluble hydroxy or lower alkoxy lower alkyl acrylate or methacrylate polymer or a copolymer of 20 to 70% of a lower acrylate or methacrylate and 80 to 30% of acrylamide, methacrylamide, N-lower alkyl acrylamide or methacrylamide, or N-vinylpyrrolidone as a powder and (b) applying, simultaneously or in succession, a high boiling liquid plasticizer or solvent therefor which does not cause a burning or stinging sensation when applied on the skin and wound to form a plastisol film on the skin resulting from adherence of the powder to the wound area wet with the non-stinging plasticizer-solvent thereby covering said wound wherein the polymer powder and plasticizer are sprayed from separate containers in succession, or wherein the polymer powder and plasticizer are simultaneously sprayed from separate chambers in a single

container, or wherein the polymer powder and plasticizer are sprayed simultaneously from the same chamber in a single container, the plasticizer and polymer powder being kept separate by the propellant which prevents solvation and agglomeration of the polymer powder by the plasticizer.

2. A method according to claim 1 wherein the polymer is in finely divided form substantially uncrosslinked and has a moisture vapor permeability of at least 200 grams/sq. meter/24 hours/mil and the application is accomplished by spraying as an aerosol with the aid of a propellant.

3. A method according to claim 2 wherein the polymer has a moisture vapor permeability of at least 500 grams/sq. meter/24 hours/mil.

4. A method according to claim 2 wherein there is included an effective amount of a medicinally active anti-septic germicide fungicide or antibiotic, local anesthetic and/or anti-inflammatory steroid ingredient in at least one of said polymer and said plasticizer, said incorporated medically active ingredients diffusing from the film to the wound area over extended periods of time, thereby keeping the wound area free from infection, inflammation, or providing local anesthesia or analgesia.

5. A method according to claim 2 wherein the polymer powder and plasticizer are sprayed from separate containers in succession.

6. A method according to claim 2 wherein the polymer and plasticizer are simultaneously sprayed from separate chambers in a single container.

7. A method according to claim 2 wherein the polymer powder and plasticizer are sprayed simultaneously from the same chamber in a single container, the plasticizer and polymer powder being kept separate by the propellant which prevents solvation and agglomeration of the polymer powder by the plasticizer prior to spraying.

8. A method according to claim 2 wherein the polymer is selected from the group consisting of polymers of hydroxy lower alkyl acrylates, hydroxy lower alkyl methacrylates.

9. A method according to claim 8 wherein the lower alkyl group has 2 to 3 carbon atoms.

10. A method according to claim 9 wherein the polymer is essentially a homopolymer of hydroxyethyl methacrylate.

11. A method according to claim 9 wherein the polymer is a copolymer of the hydroxy lower alkyl acrylate or methacrylate with each other or with up to 50% of a lower alkyl acrylate or methacrylate, a hydroxy lower alkoxy lower alkyl acrylate or methacrylate, acrylamide, methacrylamide, N-lower alkyl acrylamides and methacrylamides, lower alkoxy lower alkyl acrylates and methacrylates, diacetone acrylamide, diacetone methacrylamide, N-vinyl pyrrolidone or polymerizable amino substituted mono ethylenically unsaturated monomer.

12. A method according to claim 11 wherein the hydroxy lower alkyl acrylate or methacrylate is hydroxyethyl methacrylate.

13. A method according to claim 11 wherein there is also included in the polymerizable monomers an unsubstituted ethylenically unsaturated carboxylic acid in an amount up to 15%.

14. A method according to claim 9 wherein there is also included in the polymerizable monomers an ethylenically unsaturated carboxylic acid in an amount up to 15%.

15. A method according to claim 14 wherein the acid is selected from the group consisting of acrylic acid, methacrylic acid, maleic acid, fumaric acid and itaconic acid.

16. A method according to claim 2 wherein the polymer is a copolymer of 20 to 70% of a lower alkyl acrylate or methacrylate and 80 to 30% of a lower alkoxy lower alkyl acrylate or methacrylate, acrylamide, methacrylamide, N-lower alkyl acrylamides and methacrylamides, or N-vinyl pyrrolidone.

17. A method according to claim 1 wherein the bandage has a thickness of about 10 mils.

|           |         |                          |         |
|-----------|---------|--------------------------|---------|
| 3,269,903 | 8/1966  | Von Fieandt et al. ----- | 424—81  |
| 3,400,890 | 9/1968  | Gould -----              | 239—36  |
| 3,428,043 | 2/1969  | Shepherd -----           | 128—268 |
| 3,483,870 | 12/1969 | Coover et al. -----      | 128—334 |

## References Cited

## UNITED STATES PATENTS

|           |        |                        |        |
|-----------|--------|------------------------|--------|
| 2,542,897 | 2/1951 | Brown et al. -----     | 424—81 |
| 2,624,690 | 1/1953 | Leader -----           | 424—81 |
| 2,976,576 | 3/1961 | Gallienne et al. ----- | 424—81 |
| 2,976,576 | 3/1961 | Wichterle et al. ----- | 18—58  |
| 3,025,219 | 3/1962 | Maeder -----           | 424—81 |
| 2,976,576 | 3/1961 | Wichterle et al. ----- | 18—58  |

5 SHEP K. ROSE, Primary Examiner

U.S. CL. X.R.

424—28, 32, 33, 45, 78, 80, 81; 128—82, 114, 155, 156,  
10 172, 260, 265, 268, 334, 335.5